

Aug. 28, 1951

H. W. LEVERENZ ET AL  
MAGNETIC MATERIALS

2,565,861

Filed Sept. 26, 1947

4 Sheets-Sheet 1

Fig. 1



Inventor  
Humboldt W. Leverenz  
& Robert L. Harvey  
Attorney  
Maurice Kalman

Aug. 28, 1951

## H. W. LEVERENZ ET AL. MAGNETIC MATERIALS

**2,565,861**

Filed Sept. 26, 1947

4 Sheets-Sheet 2

Fig. 2



## Inventor

*Humboldt W. Leverenz  
& Robert L. Harvey*

Marish Rabani

Attorney

Aug. 28, 1951

H. W. LEVERENZ ET AL  
MAGNETIC MATERIALS

2,565,861

Filed Sept. 26, 1947

4 Sheets-Sheet 3

Fig. 3



Fig. 4



Fig. 5



Inventor  
Humboldt W. Leverenz  
& Robert L. Harvey

88

Marshall Hansen

Attorney

Aug. 28, 1951

H. W. LEVERENZ ET AL  
MAGNETIC MATERIALS

2,565,861

Filed Sept. 26, 1947

4 Sheets-Sheet 4

*Fig. 6*



*Fig. 6A*



*Fig. 6B*



*Fig. 6C*



Inventor  
Humboldt W. Leverenz  
& Robert L. Harvey

20

*Humboldt W. Leverenz*

Attorney

## UNITED STATES PATENT OFFICE

2,565,861

## MAGNETIC MATERIALS

Humboldt W. Leverenz and Robert L. Harvey,  
 Princeton, N. J., assignors to Radio Corpora-  
 tion of America, a corporation of Delaware

Application September 26, 1947, Serial No. 776,292

12 Claims. (Cl. 252—62.5)

1

This invention relates to improved materials having relatively high magnetic permeability and, at the same time, desirably low loss values (high Q factor) at radio frequencies and to improved articles made of these materials.

Whenever Q values are discussed or stated throughout this specification, there is meant a numerical value found by dividing the radio frequency reactance by the resistance of a circuit in which the materials of the present invention are introduced as induction coil core bodies.

The present invention is an improvement over our previous invention disclosed in application, Serial No. 719,594, filed December 31, 1946. In the said previous application, compositions comprising mainly  $Fe_2O_3$  and  $MgO$  were described. To these basic materials small amounts of other oxides, such as  $Al_2O_3$ , could be added.

It has now been found that the addition of zinc oxide to the previous reaction mixtures results in the formation of reaction products having still further improved properties as regards magnetic permeability and low loss factor. It has also been found that  $ZnO$  may be substituted for the  $MgO$ , wholly or partially, and that certain other oxides may be substituted in whole or in part for the  $ZnO$  and others for the  $MgO$ . As disclosed in our above mentioned earlier application, there may also be added small percentages of  $Al_2O_3$ ,  $Ga_2O_3$  or  $Gd_2O_3$ , or combinations of these.

One object of the present invention is to provide improved compositions having relatively high magnetic permeabilities with desirably high Q factor as well.

Another object is to provide materials having exceptionally high degrees of magnetic permeability with good temperature stability.

Another object of the invention is to provide improved materials having relatively high degrees of magnetic permeability and which can be formulated such that this permeability may have either a constant, positive, or negative temperature coefficient within the usable temperature range of the equipment.

Another object of the invention is to provide improved materials having relatively high magnetic permeabilities and which may be given positive, negative or constant coefficients of magnetostriction by proper selection of composition and temperature of crystallization.

Another object is to provide a system composed of a novel form of crystalline

2

from which may be chosen compositions having very high effective magnetic permeability, high Q factor at broadcast frequencies and excellent temperature stability.

5 Another object is to provide a novel class of compositions in the group known as ferrites, which have improved properties of both magnetic permeability and high Q factor along with other desirable properties.

10 Another object is to provide materials as above described, which can be compressed into shaped bodies before heating, to form products having greatly improved properties of magnetic permeability and high Q values of radio frequencies.

15 Still another object is to provide novel methods of preparing improved materials having high magnetic permeability or high Q value or both.

20 These and other objects will be more readily apparent and the invention will be better understood with reference to the following specification, including the drawings of which:

Fig. 1 is a graphical illustration of one modification of a system of which the compositions useful in the present invention are a part, together with indicated optimum values of magnetic permeability, without regard to optimum Q value, for compressed bodies made up of various compositions within the system.

25 Fig. 2 is a graphical illustration of the same system shown in Fig. 1 with indicated optimum values of Q factor without regard to optimum magnetic permeability for compressed bodies made up of various compositions within the system.

30 Fig. 3 is a graphical representation of data obtained by measuring the relative magnetic permeability of compressed bodies of several different compositions, within the scope of the present invention, maintained at various temperatures.

35 Fig. 4 is graphical representation of data obtained by measuring the relative magnetic permeability at various ambient temperatures of several different compressed bodies, each formed

40 at a different heating temperature but all having been formed from reaction mixtures composed of the same constituents present in the same relative molecular proportions.

45 Fig. 5 is a graph of relative Q values made for the same bodies, the permeabilities of which are shown in Fig. 4, and

50 Fig. 6, 6A, 6B and 6C are views in perspective of examples of compressed bodies made of com-

positions within the scope of the present invention.

Although the compositions, which are a part of the present invention, are different from those described in our previously mentioned co-pending application, Serial No. 719,594, the general method of preparation is the same as illustrated therein. Briefly, this method includes the intimate mixing of  $MgO$ ,  $Fe_2O_3$  and  $ZnO$ , each in a fine state of subdivision, heating, preferably, a compressed body made of these oxides within a range of temperatures of about  $900^{\circ}C$ . to  $1500^{\circ}C$ . for from 10 minutes to 2 hours in an oxidizing atmosphere and then cooling. Optimum conditions of time and temperature of heating will vary with each specific composition possible within the system of compositions which is a part of the present invention and with any one specific composition the optimum heating time decreases as the temperature of heating increases. In general, however, some improvement in results is obtained by selecting widely varying times and temperatures within the range specified even though these improvements will not be the maximum obtainable when a more careful choice is made. Good results can be expected with almost any of the compositions, if a heating time of about 1 hour is used, and a heating temperature of the order of  $1200^{\circ}C$ . has proved satisfactory, if not always best, with all of the compositions. The reaction product which is formed in all instances is a composite homogeneous crystalline body which does not have the same stoichiometric proportion of oxygen to metals as is present in the mixture before heating, but the exact proportions of the elements present in the products is not known and cannot be easily determined. Although the products resemble previously known ferrites to some extent, they are apparently different in structure, both chemically and physically, since their electrical properties are strikingly different. It is evident, for example, that the crystalline structure of these materials is novel and that the properties depend to some degree on the extent to which the crystalline structure is permitted to develop.

The oxidizing atmosphere in which the heating of the reaction mixture takes place may be supplied by passing a stream of oxygen through the reaction chamber. Less desirably, air may be used in place of oxygen. It is also possible to form products having improved magnetic permeability and low loss by heating the oxides in a neutral atmosphere, such as helium or nitrogen, but the improvement is not as great as when an oxidizing atmosphere is used. In contrast to the use of either an oxidizing or a neutral atmosphere, the presence of a reducing atmosphere, such as supplied by carbon monoxide or hydrogen, in the reaction chamber, is distinctly detrimental if materials having high permeability are desired. Therefore, it may be said that the heating should take place in a non-reducing atmosphere, preferably at atmospheric, or higher, pressures.

As pointed out in our previously mentioned co-pending application, it is possible to start with a mixture of materials in other than the oxide form in which they are present in the reaction product providing these starting materials will be changed to the specified oxide upon heating to the temperatures, times and atmospheric conditions stipulated. For example, instead of starting with a mixture containing  $Fe_2O_3$  the iron may be in the form of ferrous oxide, or magnetite, providing that heating takes place in an oxidizing atmos-

phere and as the hydroxide or carbonate, etc., if either an oxidizing or a neutral atmosphere is present. The other ingredients may also be present in forms such as hydroxides, acetates or carbonates which will revert to the desired oxide form when heated strongly in either an oxidizing or neutral atmosphere.

As previously stated, it is preferable, from a practical standpoint, to form compressed bodies of the reactants at pressures of say 20,000 p. s. i. and treat these bodies at elevated temperatures in order to impart the desired properties of increased permeability and low loss. The fact that shaped bodies of the compressed material can be formed without the presence of a permanent binder adds much to their improvement over materials previously known, such as powdered iron, which requires the use of a permanent binder, since the binder introduces a multitude of gaps of considerable size between the particles, and the gaps, themselves, are responsible for much of the lower permeability hitherto present in materials of this nature. When the material is made in the form of compressed bodies, the pressure of forming may vary widely. Pressures of 2,000 p. s. i. have been found to produce the same improved results as those ten times as great. In general, it may be said that the pressure of forming should be sufficient to form a closely coherent body.

After the heat treatment is accomplished as described, the reaction product is preferably, although not necessarily, cooled very rapidly, as by subjecting it to a blast of air or quenching in water. Rapid cooling generally increases the permeability and low loss qualities above those values obtained when slow cooling is used.

The reaction mixture may be compressed into any desired shape before heating takes place in the reaction chamber. Thus, the powder may be formed into bars having either rectangular or cylindrical cross section, into toroidal forms or into flat slabs, etc., as illustrated in Figs. 6, 6A, 6B, and 6C. When some of the forms, such as flat slabs, are heated, at the elevated temperatures required, considerable warping may ordinarily occur. It has been found possible to provide techniques for the forming of these shaped bodies in which distortion is either largely or completely eliminated. One of these techniques includes the mixing of small percentages of a lubricant with the powdered oxides and then compressing them into desired shape. The shaped body is then heated as usual and the lubricant is completely burned off. Stearic acid in percentages of about 4 or 5 percent of the oxides present has been found suitable. The percentages are not very critical. Another lubricant found usable in about the same percentages is composed of one part trigamine stearate to 4 parts of a microcrystalline wax such as Carbowax. The lubricant apparently has the function of permitting more intimate packing of the powdered oxides so that heating takes place more evenly throughout the body. Since the lubricant must be of such a nature that it is completely volatilized during the subsequent heating it does not appear in the final reaction product.

Another improvement in molding technique which was found to produce unexpectedly improved results is a feature of the present invention. The material is first placed in the mold and compressed at the usual high pressures. Then the pressure is released uniformly, as by hydraulic means, throughout the mold area.

This has been found to greatly reduce warping tendencies when the material is later heated at high temperatures and then cooled.

The manner in which the optimum magnetic permeability  $\mu$  of the compositions, made according to the present invention, varies with the proportions of the three main ingredients present in the reaction mixture is illustrated in Fig. 1. This figure, first of all, represents all possible combinations within the ternary system



Upon this system representation have been superimposed curves, each of which shows all compositions found to have a particular value of relative permeability, which value is the number given to the curve. For example, the curve designated (2) has been drawn through all points representing all compositions of the reaction mixture having a relative permeability  $\mu$  equal to 2 when the mixture is compressed and crystallized as described. Absolute permeability values  $\mu'$  are considerably in excess of those shown on the curves. All compositions tested were formed by mixing the oxides as previously described, forming each sample into a short bar  $1\frac{1}{8}$  inches long, having a cross section 0.1 inch square, by molding at 20,000 p. s. i. pressure and heating at temperatures ranging from 1100 to 1400° C. All measurements were made at room temperature of about 25° C. by inserting the bar within a uniformly wound coil slightly larger in diameter than the thickness of the bar and using a frequency of about 600 kilocycles. A powdered iron core of similar dimensions was used as a reference standard. The reference core exhibited a relative permeability  $\mu$  under similar conditions of about 5.7. The test coil, alone, which was constructed of 186 turns of No. 005 copper wire, inside diameter  $\frac{1}{4}$ ", and had a Q value of 60 and the resonant testing circuit was tuned by a shunt capacitance of  $100 \mu\text{f}$ . Samples were tested of each composition which had been fired at various temperatures within the range specified and those having the highest values of  $\mu$  for each composition were selected for purposes of illustration without regard to their Q values when tested in a resonant circuit.

It can readily be seen from the figure that those reaction mixtures having appreciable percentages of all three of the oxides produced reaction products having the highest permeability values. However, the optimum amount of ZnO to be added to the  $\text{Fe}_2\text{O}_3$ -MgO reaction mixture depends upon the relative proportions of the latter two ingredients present. Referring to curve (13) of Fig. 1, for example, it can be seen that a compressed body having a relative permeability of 13 may be constituted by the reaction product produced by treating a mixture containing the relative proportions of 0.5 mole part  $\text{Fe}_2\text{O}_3$ , 0.34 mole part MgO and 0.16 mole part ZnO. Referring to the same curve (13) it can also be seen that a product having the same relative permeability may be made from a reaction mixture made up of the relative proportions of 0.46 mole part  $\text{Fe}_2\text{O}_3$ , 0.25 mole part MgO and 0.29 mole part ZnO.

The closeness with which curves (8), (9) and (10) approach the  $\text{MgO}-\text{Fe}_2\text{O}_3$  axis brings out the fact that the addition of very small mole proportions of ZnO to the  $\text{MgO}-\text{Fe}_2\text{O}_3$  mixture produces significant increases in the permeability of the product, the lower limits of significance appearing to be about one mole per cent.

The data illustrated on Fig. 1 also show that additions of ZnO, in amounts of more than about 0.45 mole part on a basis of 0.55 mole part for the sum of the other two oxides, produces no improved results in products operated at room temperature. Stated in other terms, the upper limit of ZnO should be about 45 mole per cent of the whole composition for room-temperature (or higher) operation.

Fig. 1 also illustrates that the compositions of the present invention should contain from about 30 to about 75 mole per cent  $\text{Fe}_2\text{O}_3$ , if superior permeability is desired, although curve (6) includes compositions having slightly less than 30 mole per cent  $\text{Fe}_2\text{O}_3$ .

Compositions according to the present invention may comprise  $\text{Fe}_2\text{O}_3$  and ZnO with no MgO present. As indicated in Fig. 1, certain compositions falling on the  $\text{Fe}_2\text{O}_3$ -ZnO axis have usefully high permeabilities and some of these have desirably high Q values as well. The figure indicates that the preferred compositions in the binary system are from  $0.8\text{Fe}_2\text{O}_3 \cdot 0.2\text{ZnO}$  to about  $0.6\text{Fe}_2\text{O}_3 \cdot 0.4\text{ZnO}$ , or in other words, the reaction mixture should contain from 0.6-0.8 mole part  $\text{Fe}_2\text{O}_3$  and 0.4-0.2 mole part ZnO.

In those compositions having all three ingredients present, the amount of MgO may vary considerably, again depending upon the relative proportions of the  $\text{Fe}_2\text{O}_3$  and ZnO present. The smallest amounts of MgO which may be regarded as significant in replacing some of the ZnO is about 1 mole per cent while the highest amount of MgO found to be operative in the production of materials having high permeability is about 69 mole per cent in the ternary system. It is also apparent that MgO must be present in these compositions, providing no other oxides are considered except  $\text{Fe}_2\text{O}_3$  and ZnO, if materials having effective permeabilities of 11 or more are to be obtained.

As previously noted, the curves plotted in Fig. 1 have been drawn by selecting materials, heated within the range of 1100°-1400° C., which exhibited the highest permeability values found for each tested composition within this heating range whether a correspondingly high Q value was found or not. However, for purposes of comparison the Q values of some of the compositions have been spotted throughout the figure. These values have been indicated thus; 100, with their numerical values underlined. These values were measured as later described in connection with Fig. 2.

One general aspect of the present invention, then, is the discovery that when intimate mixtures of either  $\text{Fe}_2\text{O}_3:\text{ZnO}$  or mixtures of  $\text{Fe}_2\text{O}_3:\text{ZnO}:\text{MgO}$  are heated in a non-reducing atmosphere at from 900°-1500° C., there are formed novel crystalline products which have novel properties not found when mixtures of these oxides are heated under other conditions.

A specific aspect of the invention is the discovery that certain proportions of these oxides should be used within the ranges indicated in order to obtain products having a higher magnetic permeability than materials heretofore commonly known and used.

Within the range of compositions previously delineated as having usefully high permeabilities, there may also be selected a preferred range of compositions having unusually high permeability values which adapt these materials to uses not hitherto found practical in connection with permeable materials heretofore in use. These com-

positions are reaction products selected from Fig. 1 and are encompassed within the polygons A and B. Those within the polygon A comprise 0.45-0.55 mole part  $\text{Fe}_2\text{O}_3$  to 0.05-0.35 mole part  $\text{ZnO}$  and 0.1-0.50 mole part  $\text{MgO}$ . Those within the polygon B comprise 0.55-0.70 mole part  $\text{Fe}_2\text{O}_3$  to 0.25-0.35 mole part  $\text{ZnO}$  and 0-0.2 mole part  $\text{MgO}$ .

For many practical uses within the field of radio or, more generally, electricity, including electronics, it is highly desirable that the products should have not only high magnetic permeability but a high Q factor at radio frequencies which may range from audio frequencies up to about 5 megacycles.

Fig. 2 is a plot based on the same general system of compositions illustrated in Fig. 1, with superimposed curves, each of which is drawn through all points exhibiting the same Q value. Again, the reaction products were prepared by heating the reaction mixtures at from 1100°-1400° C. and the ones exhibiting optimum results within this range selected without regard to their permeability values. Each curve is numbered with the corresponding Q value which it represents and it is readily apparent that the curves may not be continuous. Series of compositions isolated from each other may exhibit similar Q values. In general, it has been found, as illustrated in the figure, that the same general range of compositions which have been selected as having usefully high permeabilities also exhibit usefully high Q values.

Within the broader range of compositions having usefully high Q values, there may be chosen a narrower preferred range of compositions having unusually high Q values which fit them for special applications in the electronics field. These compositions comprise 0.55-0.75 mole part  $\text{Fe}_2\text{O}_3$  to 0.01-0.40 mole part  $\text{ZnO}$  and 0.05-0.44 mole part  $\text{MgO}$ . The area representing these preferred compositions is shown by the quadrilateral A within the system diagram of Fig. 2. For purposes of illustration and for indicating the area of optimum  $\mu \times Q$  several values of permeability indicated by underlined numbers have been spotted throughout the figure.

All values shown in Fig. 2 were measured at about 600 kc., the Q value of the measuring coil alone being 62 at 2.2 megacycles and the resonant testing circuit was tuned by a shunt capacitance of  $100\mu\mu\text{f}$ . All data were also taken at room temperature of about 25° C. and the dimensions of the cores and testing coil were the same as specified in connection with the explanation of Fig. 1.

A study of Figs. 1 and 2 will show that the reaction products having the highest values of magnetic permeability do not usually have also optimum Q values. Therefore, it is not possible to pick out those compositions having the highest effective permeability, say 15, and assume that they are the optimum for given application. But since many compositions having a permeability not far below the optimum found in the system also have a reasonably high Q value, it will usually be possible to compromise on products which do have desirably high values in both respects. For example, a composition representing the reaction product of about 0.6 mole part  $\text{Fe}_2\text{O}_3$ , 0.2 mole part  $\text{MgO}$  and 0.2 mole part  $\text{ZnO}$  exhibits an effective magnetic permeability of 10 and a Q value of 118. Other compositions may be selected having still higher permeabilities and only slightly Q values.

A range of preferred compositions having an unusually high product of  $\mu \times Q$  is found within the larger system of compositions forming the basis of the present invention. These compositions are, perhaps, the most valuable of all since they readily lend themselves to applications within the field of electronics not hitherto found practical with the relatively low permeable materials previously known. This preferred range of compositions comprises 0.47-0.63 mole part  $\text{Fe}_2\text{O}_3$  to 0.04-0.29 mole part  $\text{ZnO}$  and 0.12-0.33 mole part  $\text{MgO}$  with all proportions being understood to be approximate since no sharp line of demarcation has been found. These compositions are designated in Fig. 1 by the quadrilateral C.

Another important factor to be considered in selecting materials of this nature for practical applications within the electrical field is their stability within the expected range of operating temperatures. Fig. 3 is a graph of the variation of effective permeabilities of six different compositions within certain ranges of temperature. All of the compositions selected show sharp drops in permeability value within certain narrow temperature ranges. The temperature at which this sharp drop occurs for any particular composition is known as its Curie point. The Curie point is different for each composition. It is the temperature above which thermal agitation interferes with the electron-spin orientations required for magnetism. As related to Figs. 1 and 2, all of the compositions plotted in Fig. 3 lie along the horizontal line 4.5-4.5 but the heating temperature in all cases was 1100° C. The relative proportions of each composition are expressed in mole parts.

Table of compositions plotted in Fig. 3

|   | Curve | $\text{Fe}_2\text{O}_3$ | $\text{MgO}$ | $\text{ZnO}$ |
|---|-------|-------------------------|--------------|--------------|
| A |       | 1.0                     | 1.0          | 0.2          |
| B |       | 1.0                     | 0.8          | 0.4          |
| C |       | 1.0                     | 0.6          | 0.6          |
| D |       | 1.0                     | 0.5          | 0.7          |
| E |       | 1.0                     | 0.4          | 0.8          |
| F |       | 1.0                     | 0.3          | 0.9          |

It is apparent that a given material should be used at temperatures below its Curie point if temperature stability is to be expected.

Another aspect of the invention is the discovery that the temperature of crystallizing the reaction product greatly influences the later performance of the material when it is subjected to changes in the ambient temperature. With any particular composition, it is possible to find, by experimenting with different temperatures of heating within the range previously specified, a preferred heating temperature which will produce a product that will have a substantially constant permeability as a function of the ambient operating temperature from 20°-80° C. It has also been found possible with a particular composition to find temperatures of heating which will produce reaction products having either positive or negative temperature coefficients of permeability. This is illustrated in Fig. 4. In this figure, all curves show effective permeability plotted against change in ambient temperature for a reaction product made by mixing ferric, magnesium and zinc oxides in the proportion  $\text{Fe}_2\text{O}_3:0.5\text{MgO}:0.5\text{ZnO}$  and crystallizing in an oxidizing atmosphere at three different temperatures. Curve (A) is a record of

the variation in magnetic permeability of a core of the compressed reaction product, made up and tested as previously described, when the crystallizing temperature was 1100° C. Curves (B) and (C) are similar curves plotted from cores heated at 1200° C. and 1300° C., respectively. The data shown in the figure illustrate the fact that a core of this particular composition prepared at a heating temperature of 1200° C. shows a substantially zero temperature coefficient of permeability between 20° and 80° C. and that, therefore, this crystallizing temperature should be approximately adhered to, if good temperature stability is desired in the reaction product prepared from this particular composition. The figure also shows that cores of the same composition crystallized at 1100° C. exhibit negative temperature coefficients of permeability and those crystallized at 1300° C. exhibit positive coefficients. It should be understood, however, that these temperatures are approximate, only, and that differences of a few degrees, either way, in the heating temperature will produce no significant changes in results. It should also be understood that the critical values will be different for different compositions and that the preferred values for any one composition can only be determined by experiment. In the examples illustrated, the time of heating was selected to produce materials having optimum permeability but other heating temperatures within the median range give approximately the same results in this respect.

Figure 5 is a plot of the relative Q values for the same cores, testing data for which are shown in Fig. 4, curve (D) being a plot of relative Q value as a function of ambient operating temperatures from 20°-80° C. for the core crystallized at 1100° C. and curves (E) and (F) being test data obtained by measuring cores of the same initial composition heated at 1200° C. and 1300° C., respectively. It is noted that all cores having this composition exhibit negative temperature coefficients with respect to their Q values within the operating temperature range specified, although the coefficients differ one from another. It has been found, additionally, that all cores do not exhibit negative coefficients when those of different compositions are tested. For example, a core made up of a starting mixture of  $Fe_2O_3:1.2MgO$  showed all positive coefficients with regard to the Q value.

In addition to the control of the temperature coefficients of permeability and Q values described above, it has also been found possible to provide materials having either positive, negative or constant coefficients of magnetostriction by proper choice of composition and crystallization temperature in the  $Fe_2O_3:MgO:ZnO$  system. As an example, in the system

#### $Fe_2O_3:MgO:ZnO$

those compositions containing about 0.5-0.75 mole part  $Fe_2O_3$  to 0.5-0.25 mole part of the sum of the other two oxides have been observed to have positive values of magnetostriction while those compositions having less than 50 mole per cent  $Fe_2O_3$  tend to have negative values of magnetostriction. For most practical applications, therefore, it is desirable to choose compositions within the former range when magnetostrictive properties are important.

Although, in the present invention, it is preferred to use compositions containing the 3 oxides  $MgO$ ,  $ZnO$  and  $Fe_2O_3$ , it has been found

possible to substitute  $CdO$  for some or all of the  $ZnO$  in this system. The preparation of the materials is carried out in exactly the same manner as when  $ZnO$  is used and the preferred proportions of  $CdO$  fall within approximately the same limits as found for  $ZnO$ . The permeability values and Q values may be described as comparable although somewhat inferior to those found for compositions in which no  $CdO$  is used.

Another substitution which may be made within the scope of the present invention is the substitution of  $NiO$  in whole or in part for  $MgO$ . In a binary system containing only  $Fe_2O_3$  and  $NiO$ , the preferred proportions of the ingredients are 0.4-0.53 mole part  $Fe_2O_3$  to 0.6-0.47 mole part  $NiO$ . This range is found by inspection of the  $MgO-Fe_2O_3$  axis of Fig. 1 since the  $NiO$  may be substituted for the  $MgO$  without appreciable change in proportions. Although the usual chemical properties of magnesium and nickel differ widely, their ionic radii are about the same. Hence, in a crystalline network, nickelous ions would occupy about the same space dimensions as magnesium ions and this appears to account for the similarity of their electrical properties in the compositions of the present invention. As described in the previously mentioned co-pending application, Serial No. 719,594, there may be added small percentages of trivalent oxides from the class consisting of  $Al_2O_3$ ,  $Ga_2O_3$  and  $Gd_2O_3$  to provide additional small improvements in permeability values and in other operating characteristics. The preferred range of amounts of the addition agents used is 0.01 to 0.10 mole, expressed as oxide, per mole  $Fe_2O_3$  present. A preferred composition was made up by mixing 1 mole part  $Fe_2O_3$ , 0.5 mole part  $MgO$ , 0.5 mole part  $ZnO$  and .015 mole part  $Al(OH)_3$ , heating at 1100° C. for 1 hour in compressed core form and cooling. The core had a relative permeability of 16 and a Q value of 35.

There has thus been described a series of novel crystalline materials having strikingly improved properties with respect to magnetic permeability, Q value, and magnetostriction, which properties greatly enhance their value and broaden the scope of use of this class of material in the electronics field. Although several embodiments of our invention have been described, it will undoubtedly be apparent to those skilled in the art that equivalent forms are possible.

We claim as our invention:

1. An article of manufacture characterized by having a high effective magnetic permeability comprising a compressed body made up of a reaction product produced by heating an intimate mixture of 1 mole part  $Fe_2O_3$ , 0.5 mole part  $MgO$ , 0.5 mole part  $ZnO$  and 0.015 mole part  $Al(OH)_3$  at about 1400° C. for about 1 hour in an oxidizing atmosphere.

2. A composition of matter consisting essentially of the reaction product produced by heating together in a non-reducing atmosphere at temperatures of from 900°-1500° C. for from 10 minutes to 2 hours, an intimate mixture of 0.3-0.75 mole part  $Fe_2O_3$ , 0.01-0.69 mole part of a second ingredient which is at least one of a class consisting of magnesium and nickel oxides and 0.01-0.45 mole part of a third ingredient which is a mixture of zinc and cadmium oxides.

3. A composition according to claim 2 in which the proportions of the oxides in the reaction mixture comprise 0.45-0.55 mole part  $Fe_2O_3$  to 0.10-0.5 mole part of said second ingredient and 0.05-0.35 mole part of said third ingredient.

11

4. A composition according to claim 2 in which the proportions of the oxides of the reaction mixture comprise 0.55-0.75 mole part  $Fe_2O_3$  to 0.05-0.44 mole part of said second ingredient and 0.01-0.4 mole part of said third ingredient.

5. A composition according to claim 2 in which the proportions of the oxides of the reaction mixture comprise 0.47-0.63 mole part  $Fe_2O_3$  to 0.12-0.30 mole part of said second ingredient and 0.12-0.3 mole part of said third ingredient.

6. A composition of matter consisting essentially of the reaction product produced by heating together in a non-reducing atmosphere at a temperature of from 900° C. to 1500° C. for from ten minutes to two hours, an intimate mixture of 0.3-0.75 mole part ferric oxide, 0.01-0.69 mole part of a second ingredient which is at least one of a class consisting of magnesium and nickel oxides, 0.01-0.45 mole part of a third ingredient which is at least one of a class consisting of zinc and cadmium oxides and 0.01-0.10 mole part of a fourth ingredient which is at least one of a class consisting of aluminum, gallium and gadolinium oxides.

7. A molded body of predetermined shape consisting essentially of a reaction product produced by heating together in a non-reducing atmosphere at a temperature between 900° and 1500° C. for from 10 minutes to 2 hours, an intimate mixture of 0.3-0.75 mole part  $Fe_2O_3$ , 0.01-0.69 mole part of a second ingredient which is at least one of a class consisting of magnesium and nickel oxides and 0.01-0.45 mole part of a third ingredient which is a mixture of zinc and cadmium oxides.

8. A molded body according to claim 7 in which said second ingredient is magnesium oxide.

9. A molded body according to claim 7 in which said second ingredient is nickel oxide.

10. A molded body according to claim 7 in

which said second ingredient is a mixture of magnesium and nickel oxides.

11. A molded body of predetermined shape consisting essentially of a reaction product produced by heating together in a non-reducing atmosphere at a temperature between 900° and 1500° C. for from 10 minutes to 2 hours, an intimate mixture of 0.3-0.75 mole part  $Fe_2O_3$ , 0.01-0.69 mole part of a mixture of magnesium and nickel oxides, and 0.01-0.45 mole part zinc oxide.

12. A molded body of predetermined shape consisting essentially of a reaction product produced by heating together in a non-reducing atmosphere at a temperature between 900° and 1500° C. for from 10 minutes to 2 hours, an intimate mixture of 0.3-0.75 mole part  $Fe_2O_3$ , 0.01-0.69 mole part of a mixture of magnesium and nickel oxides, and 0.01-0.45 mole part cadmium oxide.

HUMBOLDT W. LEVERENZ.  
ROBERT L. HARVEY.

#### REFERENCES CITED

The following references are of record in the file of this patent:

#### UNITED STATES PATENTS

| Number    | Name  | Date          |
|-----------|-------|---------------|
| 1,946,964 | Cobb  | Feb. 13, 1934 |
| 1,976,230 | Kato  | Oct. 9, 1934  |
| 2,068,658 | Cox   | Jan. 26, 1937 |
| 2,452,529 | Snoek | Oct. 26, 1948 |

#### OTHER REFERENCES

Magnetic and Electrical Properties of the Binary Systems  $MO-Fe_2O_3$  by J. L. Snoek published in *Physica III*, No. 6, June 1936, pages 481 and 482.